



US006037113A

# United States Patent [19]

Shuttleworth et al.

[11] Patent Number: 6,037,113

[45] Date of Patent: Mar. 14, 2000

[54] **PHOTOGRAPHIC ELEMENT AND PROCESS FOR ITS USE**

91/14970 10/1991 WIPO .

[75] Inventors: **Leslie Shuttleworth**, Webster, N.Y.; **Rakesh Jain**, Cupertino, Calif.; **John W. Harder**, Rochester, N.Y.

Primary Examiner—Geraldine Letscher  
Attorney, Agent, or Firm—Arthur E. Kluegel

[73] Assignee: **Eastman Kodak Company**, Rochester, N.Y.

## [57] ABSTRACT

Disclosed is a photographic element comprising a light sensitive silver halide emulsion layer having in association therewith at least one dye-forming coupler of Formula (1a):

[21] Appl. No.: 09/134,846

(1a)

[22] Filed: Aug. 14, 1998

[51] Int. Cl.<sup>7</sup> ..... G03C 1/08; G03C 7/26; G03C 7/32

[52] U.S. Cl. ..... 430/558; 430/551; 430/955; 430/372; 430/386; 430/387

[58] Field of Search ..... 430/306, 307, 430/543, 558, 955, 551, 372



## [56] References Cited

### U.S. PATENT DOCUMENTS

- |           |         |                |       |         |
|-----------|---------|----------------|-------|---------|
| 4,338,393 | 7/1982  | Bailey et al.  | ..... | 430/558 |
| 4,360,589 | 11/1982 | Kojima et al.  | ..... | 430/551 |
| 4,880,733 | 11/1989 | Kaneko         | ..... | 430/551 |
| 5,063,148 | 11/1991 | Sugita et al.  | ..... | 430/551 |
| 5,143,821 | 9/1992  | Crawley et al. | ..... | 430/387 |
| 5,561,037 | 10/1996 | Jain et al.    | ..... | 430/551 |
| 5,776,669 | 7/1998  | Crawley et al. | ..... | 430/558 |
| 5,876,912 | 3/1999  | Crawley et al. | ..... | 430/558 |

### FOREIGN PATENT DOCUMENTS

1 529 908 10/1978 United Kingdom .

wherein:

R<sub>1</sub> is an alpha-branched alkyl group with greater than 10 carbon atoms;

R<sub>5</sub>, R<sub>6</sub>, R<sub>7</sub>, and R<sub>8</sub> are each independently a hydrogen atom or a substituent;

Z is a hydrogen atom or a group which can be split off by the reaction of the coupler with an oxidized color developing agent.

The element exhibits improved dye light stability.

**15 Claims, No Drawings**

**PHOTOGRAPHIC ELEMENT AND PROCESS  
FOR ITS USE**

**FIELD OF THE INVENTION**

The present invention relates to a color photographic element comprising a light-sensitive silver halide emulsion layer having associated therewith a pyrazolo[1,5-a]benzimidazole coupler having an alpha branched alkyl group with greater than 10 carbon atoms in the 2-position.

**BACKGROUND OF THE INVENTION**

Silver halide color photography depends on the formation of dyes in order to reproduce an image. These dyes are typically formed from couplers present in or adjacent to the light sensitive silver halide emulsion layers which react to image light upon exposure. During development, the latent image recorded by the silver halide emulsion is developed to amplify the image. During this process in which silver halide is reduced to elemental silver, the color developer compound used is at the same time oxidized, as is typical in a redox reaction. The oxidized developer then reacts or couples with the coupler compound present in or adjacent to the emulsion layer to form a dye of the desired color.

Typically, a silver halide emulsion layer containing a magenta dye-forming coupler is sensitized to green light. This facilitates so-called negative-positive processing in which the image is initially captured in a negative format where black is captured as white, white as black, and the colors as their complimentary colors (e.g., green as magenta, blue as yellow, and red as cyan). Then the initial image can be optically printed in the correct colors on a reflective background through the device of optical printing which has the effect of producing a negative of the negative, or a positive image of the original scene.

Viewable images may also be produced through reversal processing in which the initial negative image is reversed by using a black and white developer, processing to remove the developed silver but leave the undeveloped silver halide, and then fogging the element in the presence of color developer to provide developed silver in inverse proportion to the amount of image light, with corresponding dye formation.

For incorporation into a photographic element, the couplers are typically dissolved in high-boiling organic solvents known as "coupler solvents," and dispersed in gelatin with the aid of surfactants.

One of the difficulties with color couplers is achieving simultaneously all of the required physical and chemical properties of the coupler and the dye formed from it. For instance, the coupler must have good solubility in the coupler solvent, good dispersibility in gelatin, and high dye-forming activity. It must also have a high degree of resistance to decomposition due to light, heat and humidity, which can cause stains. The image dye must have the proper hue and must have a high degree of resistance to fading or hue changes due to light, heat and humidity.

Couplers that form magenta dyes upon reaction with oxidized color developing agent are described in such representative patents and publications as: U.S. Pat. Nos. 2,311,082, 2,343,703, 2,369,489, 2,600,788, 2,908,573, 3,062,653, 3,152,896, 3,519,529, 3,758,309, and 4,540,654; and "Farbkupplereine Literature Ubersicht," published in Agfa Mitteilungen, Band III, pp. 126-156 (1961). Typically, such couplers are pyrazolones and pyrazoloazoles, especially pyrazolo[2,3-b][1,2,4]triazoles described by Formula (A)

and pyrazolo[3,2-c][1,2,4]triazoles described by Formula (B).



In Formulas (A) and (B), R and R<sub>2</sub> represent substituents and Z is a hydrogen atom or a group capable of being split off during the coupling reaction. Typically, R<sub>2</sub> is an alkyl group. An alkoxy group in this position leads to image dyes with very poor light stability.

The present invention is concerned with the pyrazolo[1,5-a]benzimidazole type of magenta dye-forming couplers (hereafter referred to as PBI couplers). These couplers may be described by Formula (1):



in which R<sub>2</sub> and R<sub>5</sub>-R<sub>8</sub> represent hydrogen or substituents and Z represents a hydrogen atom or a group capable of being split off during the coupling reaction.

German patent 1,070,030 discloses PBI couplers that form magenta dyes upon coupling. In the examples given, R<sub>2</sub> represents an alkyl or phenyl group. Couplers of these types are known to have poor coupling reactivity and to yield image dyes whose absorption spectra are too bathochromic for practical use in color photographic papers, and which have poor stability to light. International Patent Application WO 91/14970 describes PBI couplers with specifically substituted alkylthio coupling-off groups, including carboxyalkylthio groups. Such couplers offer marked improvements in coupling reactivity but do not offer improved dye hue or light stability. U.S. Pat. No. 5,143,821 discloses PBI couplers in which R<sub>2</sub> represents an alkoxy group. Such couplers are advantageous because they have much better coupling reactivity than those in which R<sub>2</sub> represents an alkyl group, and the image dyes formed from them have good spectral absorption characteristics. The dyes from these couplers have better light stability than the dyes from PBI couplers in which R<sub>2</sub> is an alkyl group; however, the light stability of the dyes from these alkoxy PBI couplers is still not sufficient to meet the stringent requirements of future photographic products, especially color photographic papers.

Many classes of compounds are known to improve the light stability of image dyes when incorporated in the photographic element in combination with the coupler. Examples of such "light stabilizers" or "discoloration

inhibitors," as they are commonly known, are 6-hydroxychromans as described, for example in U. S. Pat. No. 3,467,772; spiroindanes as described, for example in U. S. Pat. No. 4,360,589; methylenebisphenols as described, for example in British patent 1,529,908, U. S. Pat. Nos. 3,770,455, and 5,063,148; and so forth. However, none of these types of stabilizers have been found to provide sufficient improvement in the light stability of image dyes from PBI couplers to meet the stringent requirements of future photographic products, especially color photographic papers.

Light stabilizers of the type represented by Formula (S) are disclosed in U.S. Pat. No. 4,880,733 and U.S. Pat. No. 5,561,037. The substituents  $Z_1$  and  $Z_2$  are alkylene groups of 1–3 carbon atoms such that together they contain 3 to 6 carbon atoms, and  $R_3$  is an aryl or heterocyclic group, where  $q$  is 1 or 2.



One of the embodiments of the stabilizer of Formula (S) is the thiomorpholinedioxide represented by Formula (S-1):



wherein  $R^{1'}$  is alkyl;  $R^{1''}$  is alkyl, alkoxy, alkylthio, amido, ureido or halogen;  $x$  is 0 to 4; and  $y$  is 1 or 2.

U.S. Pat. No. 5,561,037 also discloses the use of co-stabilizers of Formula I:



wherein each  $R_4$  independently represents an alkyl or alkoxy group of 1 to 32 carbon atoms and  $p$  is 1 to 4;  $Y$  is  $-\text{NHSO}_2-$  or  $-\text{SO}_2\text{NH}-$ , and  $R_5$  is an alkyl group of 1 to 16 carbon atoms.

A problem to be solved is to provide a photographic element containing a light-sensitive silver halide emulsion layer having associated therewith a pyrazolo[1,5-a] benzimidazole type of magenta dye-forming coupler that yields a magenta dye with improved stability to light.

## SUMMARY OF THE INVENTION

The invention provides a photographic element comprising a light sensitive silver halide emulsion layer having in association therewith at least one dye-forming coupler of Formula (1a):

(1a)



wherein:

$R_1$  is an alpha-branched alkyl group with greater than 10 carbon atoms;

$R_5$ ,  $R_6$ ,  $R_7$ , and  $R_8$  are each independently a hydrogen atom or a substituent;

$Z$  is a hydrogen atom or a group which can be split off by the reaction of the coupler with an oxidized color developing agent.

The invention also provides an imaging process for forming an image in the element of the invention.

The element of the invention exhibits improved magenta dye-light stability.

## DETAILED DESCRIPTION OF THE INVENTION

The coupler of the invention is more particularly described by Formula (1a).



In Formula (1a),  $R_1$  is an alpha-branched alkyl group of greater than 10 carbon atoms (including cyclic, saturated or unsaturated; and further substituted groups). Groups are defined hereinafter to include substituted or unsubstituted forms of substitutable groups.  $R_1$  represents an alkyl group in which the first carbon atom has no more than one hydrogen atom attached, such as a secondary, tertiary or cyclic alkyl group. Substituents on  $R_1$  may be any substituent as described hereinafter which is not incompatible with the intended use of the coupler. Examples of such useful substituents include, but are not limited to, an alkyl group (including linear, further branched, cyclic, saturated, unsaturated, substituted and unsubstituted), a substituted or unsubstituted aryl group, a halogen atom (e.g. Cl, Br or F), a nitro group, a cyano group, a hydroxyl group, an alkoxy group, an alkyl or aryl sulfonyl group, a substituted or unsubstituted sulfamoyl group, a substituted or unsubstituted carbamoyl group, an alkyl or aryl carbonamido group, an alkyl or aryl sulfonamido group, a carboxy group, a carboalkoxy or carboaryloxy group, a substituted or unsubstituted amino group, an alkylthio group, or an arylthio group.

$R_5$ ,  $R_6$ ,  $R_7$ , and  $R_8$  each independently represent a hydrogen atom or any of the substituents described hereinafter. Preferably,  $R_5$ ,  $R_6$ ,  $R_7$ , and  $R_8$  is each a hydrogen atom.

$Z$  represents a hydrogen atom or a group that can be split off by the reaction of the coupler with an oxidized color

5

developing agent, known in the art as a "coupling-off" group. Typical coupling-off groups are halogen atoms and aliphatic, aromatic or heterocyclic groups attached to the coupling site by means of an oxygen, sulfur or nitrogen atom. Suitably, Z is an alkylthio group which may be substituted as described in International Patent Application WO 91/14970. Suitably, Z is a carboxyalkylthio group.

Coupling-off groups can determine the chemical equivalency of a coupler, i.e., whether it is a 2-equivalent or 4-equivalent coupler, or modify the reactivity of the coupler. Such groups can advantageously affect the layer in which the coupler is coated or other layers in the photographic recording material by performing, after release from the coupler, functions such as dye formation, dye hue adjustment, development acceleration or inhibition, bleach acceleration or inhibition, electron transfer facilitation, color correction, and the like.

The presence of hydrogen at the coupling site (the site on the coupler molecule at which Z is attached) provides a 4-equivalent coupler, and the presence of a coupling-off group other than hydrogen usually provides a 2-equivalent coupler. Representative classes of such coupling-off groups include, for example, chloro, alkoxy, aryloxy, heterocyclyloxy, sulfonyloxy, acyloxy, acyl, heterocyclyl, sulfonamido, heterocyclylthio, benzothiazolyl, phosphonyloxy, alkylthio, arylthio, and arylazo. These coupling-off groups are described in the art, for example, in U. S. Pat. Nos. 2,455,169, 3,227,551, 3,432,521, 3,467,563, 3,617,291, 3,880,661, 4,052,212, and 4,134,766; and in U. K. Patents and published applications 1,466,728, 1,531,927, 1,533,039, 2,066,755A, and 2,017,704A, the disclosures of which are incorporated herein by reference.

The following examples further illustrate the coupler of the invention:

6

-continued



M5



M6



M7



M8



40



MS



M4



M9



7

-continued





(ST-III)

-continued

ST-7



ST-8



ST-9



ST-10



ST-11



ST-12



ST-13



ST-14



ST-15



ST-16



wherein  $R_a$  is an alkyl group which may be linear or branched, saturated or unsaturated, substituted or unsubstituted,  $R_b$  is a substituent,  $n$  is an integer from 0 to 4,  $R_d$  and  $R_e$  are each hydrogen atoms or alkyl groups, and any of the groups  $R_b$ ,  $R_d$  and  $R_e$  may be joined together to form a ring.

A particular embodiment is represented by Formula (ST-IV):



(ST-IV)

20

25

The following examples further illustrate this type of stabilizer. It is not to be construed that the present invention is limited to these examples.

ST-1



35

ST-2



40

ST-3



45

ST-4



50



55



60



65

In addition to the stabilizer of the preceding formulas, a co-stabilizer represented by formula (AST) is also useful:



wherein

each R<sub>4</sub> independently represents an alkyl or alkoxy group of 1 to 32 carbon atoms and p is 1 to 4;

Y is —NHSO<sub>2</sub>— or —SO<sub>2</sub>NH—, and

R<sub>5</sub> is an alkyl group of 1 to 16 carbon atoms.

Desirably, the compound is ballasted so as not to diffuse from the element during processing and suitably contains at least 8 aliphatic carbon atoms.

Suitable examples are:



AST-1



AST-2



AST-3



AST-4



AST-5



AST-6

AST

5

10

15

20

25

30

35

40

45

50

55

60

65

-continued

AST-7



AST-8



AST-9



Unless otherwise specifically stated, the term substituted or substituent means any group or atom other than hydrogen bonded to the remainder of a molecule. Additionally, when the term "group" is used, it means that when a substituent group contains a substitutable hydrogen, it is also intended to encompass not only the substituent's unsubstituted form, but also its form further substituted with any substituent group or groups as herein mentioned, so long as the substituent does not destroy properties necessary for photographic utility. Suitably, a substituent group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain or cyclic alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolylxy; carbonamido, such as acetamido, benzamido, butyramido, tetradecanamido, alpha-(2,4-di-t-pentyl-phenoxy)acetamido, alpha-(2,4-di-t-pentylphenoxy)butyramido, alpha-(3-pentadecylphenoxy)-hexanamido, alpha-(4-hydroxy-3-t-butylphenoxy)tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzoyloxycarbonylamino, hexadecyloxycarbonylamino, 2,4-di-t-butylphenoxy carbonylamino, phenylcarbonylamino, 2,5-(di-t-pentylphenyl) carbonylamino, p-dodecyl-phenylcarbonylamino, p-tolylcarbonylamino, N-methylureido, N,N-dimethylureido, N-methyl-N-dodecylureido, N-hexadecylureido, N,N-dioctadecylureido, N,N-diocetyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as methylsulfonamido, benzenesulfonamido, p-dodecylbenzenesulfonamido, N-methyltetradecylsulfonamido, N,N-

dipropylsulfamoylamino, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diocetylcarbamoyl; acyl, such as acetyl, (2,4-di-t-amylphenoxy)acetyl, phenoxy carbonyl, p-dodecyloxyphenoxy carbonyl methoxycarbonyl, butoxycarbonyl, tetradecyloxy carbonyl, ethoxycarbonyl, benzyloxycarbonyl, 3-pentadecyloxy carbonyl, and dodecyloxy carbonyl; sulfonyl, such as methoxysulfonyl, 15 octyloxysulfonyl, tetradecyloxysulfonyl, 2-ethylhexyloxysulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; 20 thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acetoxy, benzoxyloxy, octadecanoxyloxy, p-dodecylamido benzoyloxy, N-phenylcarbamoyloxy, N-ethylcarbamoyloxy, and cyclohexylcarbonyloxy; amine, such as phenylanilino, 2-chloroanilino, diethylamine, dodecylamine; imino, such as 1 (N-phenylimido)ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

The materials of the invention can be used in any of the ways and in any of the combinations known in the art. Typically, the invention materials are incorporated in a silver halide emulsion and the emulsion coated as a layer on a support to form part of a photographic element. Alternatively, they can be incorporated at a location adjacent to the silver halide emulsion layer where, during development, they will be in reactive association with development products such as oxidized color developing agent. Thus, as used herein, the term "associated" signifies that the compound is in the silver halide emulsion layer or in an adjacent location where, during processing, it is capable of reacting with silver halide development products.

To control the migration of various components, it may be desirable to include a high molecular weight hydrophobe or

"ballast" group in the component molecule. Representative ballast groups include substituted or unsubstituted alkyl or aryl groups containing 8 to 40 carbon atoms. Representative substituents on such groups include alkyl, aryl, alkoxy, aryloxy, alkylthio, hydroxy, halogen, alkoxy carbonyl, aryloxy carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 40 carbon atoms. Such substituents can also be further substituted.

The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

If desired, the photographic element can be used in conjunction with an applied magnetic layer as described in *Research Disclosure*, November 1992, Item 34390 published by Kenneth Mason Publications, Ltd., Dudley Annex, 12a North Street, Emsworth, Hampshire PO10 7DQ, ENGLAND, or as described in Hatsumi Kyousai Koukai Gihou No. 94-6023, published Mar. 15, 1994, available from the Japanese Patent Office, the contents of which are incorporated herein by reference.

In the following discussion of suitable materials for use in the emulsions and elements of this invention, reference will be made to *Research Disclosure*, September 1996, Item 38957, available as described above, which will be identified hereafter by the term "Research Disclosure". The contents of the *Research Disclosure*, including the patents and publications referenced therein, are incorporated herein by reference, and the Sections hereafter referred to are Sections of the *Research Disclosure*.

The silver halide emulsions employed in the elements of this invention can be either negative-working or positive-working. Suitable emulsions and their preparation as well as methods of chemical and spectral sensitization are described in Sections I through V. Various additives such as UV dyes, brighteners, antifoggants, stabilizers, light absorbing and scattering materials, and physical property modifying addenda such as hardeners, coating aids, plasticizers, lubricants and matting agents are described, for example, in Sections II and VI through VIII. Color materials are described in Sections X through XIII. Suitable methods for incorporating couplers and dyes, including dispersions in organic solvents, are described in Section X(E). Scan facilitating is described in Section XIV. Supports, exposure, development systems, and processing methods and agents are described in Sections XV to XX. Certain desirable photographic elements and processing steps are described in *Research Disclosure*, Item 37038, February 1995.

Image dye-forming couplers may be included in the element such as couplers that form cyan dyes upon reaction

with oxidized color developing agents which are described in such representative patents and publications as: "Farbkuppler-eine Literature Ubersicht," published in Agfa Mitteilungen, Band III, pp. 156-175 (1961) as well as in U.S. Pat. Nos. 2,367,531; 2,423,730; 2,474,293; 2,772,162; 2,895,826; 3,002,836; 3,034,892; 3,041,236; 4,333,999; 4,746,602; 4,753,871; 4,770,988; 4,775,616; 4,818,667; 4,818,672; 4,822,729; 4,839,267; 4,840,883; 4,849,328; 4,865,961; 4,873,183; 4,883,746; 4,900,656; 4,904,575; 4,916,051; 4,921,783; 4,923,791; 4,950,585; 4,971,898; 4,990,436; 4,996,139; 5,008,180; 5,015,565; 5,011,765; 5,011,766; 5,017,467; 5,045,442; 5,051,347; 5,061,613; 5,071,737; 5,075,207; 5,091,297; 5,094,938; 5,104,783; 5,178,993; 5,813,729; 5,187,057; 5,192,651; 5,200,305; 5,202,224; 5,206,130; 5,208,141; 5,210,011; 5,215,871; 5,223,386; 5,227,287; 5,256,526; 5,258,270; 5,272,051; 5,306,610; 5,326,682; 5,366,856; 5,378,596; 5,380,638; 5,382,502; 5,384,236; 5,397,691; 5,415,990; 5,434,034; 5,441,863; EPO 0 246 616; EPO 0 250 201; EPO 0 271 323; EPO 0 295 632; EPO 0 307 927; EPO 0 333 185; EPO 0 378 898; EPO 0 389 817; EPO 0 487 111; EPO 0 488 248; EPO 0 539 034; EPO 0 545 300; EPO 0 556 700; EPO 0 556 777; EPO 0 556 858; EPO 0 569 979; EPO 0 608 133; EPO 0 636 936; EPO 0 651 286; EPO 0 690 344; German OLS 4,026,903; German OLS 3,624,777, and German OLS 3,823,049. Typically such couplers are phenols, naphthols, or pyrazoloazoles.

Couplers that form magenta dyes upon reaction with oxidized color developing agent are described in such representative patents and publications as: "Farbkuppler-eine Literature Ubersicht," published in Agfa Mitteilungen, Band III, pp. 126-156 (1961) as well as U.S. Pat. Nos. 2,311,082 and 2,369,489; 2,343,701; 2,600,788; 2,908,573; 3,062,653; 3,152,896; 3,519,429; 3,758,309; 3,935,015; 4,540,654; 4,745,052; 4,762,775; 4,791,052; 4,812,576; 4,835,094; 4,840,877; 4,845,022; 4,853,319; 4,868,099; 4,865,960; 4,871,652; 4,876,182; 4,892,805; 4,900,657; 4,910,124; 4,914,013; 4,921,968; 4,929,540; 4,933,465; 4,942,116; 4,942,117; 4,942,118; U.S. Pat. Nos. 4,959,480; 4,968,594; 4,988,614; 4,992,361; 5,002,864; 5,021,325; 5,066,575; 5,068,171; 5,071,739; 5,100,772; 5,110,942; 5,116,990; 5,118,812; 5,134,059; 5,155,016; 5,183,728; 5,234,805; 5,235,058; 5,250,400; 5,254,446; 5,262,292; 5,300,407; 5,302,496; 5,336,593; 5,350,667; 5,395,968; 5,354,826; 5,358,829; 5,368,998; 5,378,587; 5,409,808; 5,411,841; 5,418,123; 5,424,179; EPO 0 257 854; EPO 0 284 240; EPO 0 341 204; EPO 347,235; EPO 365,252; EPO 0 422 595; EPO 0 428 899; EPO 0 428 902; EPO 0 459 331; EPO 0 467 327; EPO 0 476 949; EPO 0 487 081; EPO 0 489 333; EPO 0 512 304; EPO 0 515 128; EPO 0 534 703; EPO 0 554 778; EPO 0 558 145; EPO 0 571 959; EPO 0 583 832; EPO 0 583 834; EPO 0 584 793; EPO 0 602 748; EPO 0 602 749; EPO 0 605 918; EPO 0 622 672; EPO 0 622 673; EPO 0 629 912; EPO 0 646 841; EPO 0 656 561; EPO 0 660 177; EPO 0 686 872; WO 90/10253; WO 92/09010; WO 92/10788; WO 92/12464; WO 93/01523; WO 93/02392; WO 93/02393; WO 93/07534; UK Application 2,244,053; Japanese Application 03192-350; German OLS 3,624,103; German OLS 3,912,265; and German OLS 40 08 067. Typically such couplers are pyrazolones, pyrazoloazoles, or pyrazolobenzimidazoles that form magenta dyes upon reaction with oxidized color developing agents.

Couplers that form yellow dyes upon reaction with oxidized color developing agent are described in such representative patents and publications as: "Farbkuppler-eine Literature Ubersicht," published in Agfa Mitteilungen, Band In; pp. 112-126 (1961); as well as U.S. Pat. Nos. 2,298,443; 2,407,210; 2,875,057; 3,048,194; 3,265,506; 3,447,928; 4,022,620; 4,443,536; 4,758,501; 4,791,050; 4,824,771; 4,824,773; 4,855,222; 4,978,605; 4,992,360; 4,994,361; 5,021,333; 5,053,325; 5,066,574; 5,066,576; 5,100,773;

5,118,599; 5,143,823; 5,187,055; 5,190,848; 5,213,958; 5,215,877; 5,215,878; 5,217,857; 5,219,716; 5,238,803; 5,283,166; 5,294,531; 5,306,609; 5,328,818; 5,336,591; 5,338,654; 5,358,835; 5,358,838; 5,360,713; 5,362,617; 5,382,506; 5,389,504; 5,399,474; 5,405,737; 5,411,848; 5,427,898; EPO 0 327 976; EPO 0 296 793; EPO 0 365 282; EPO 0 379 309; EPO 0 415 375; EPO 0 437 818; EPO 0 447 969; EPO 0 542 463; EPO 0 568 037; EPO 0 568 196; EPO 0 568 777; EPO 0 570 006; EPO 0 573 761; EPO 0 608 956; EPO 0 608 957; and EPO 0 628 865. Such couplers are typically open chain ketomethylene compounds.

Couplers that form colorless products upon reaction with oxidized color developing agent are described in such representative patents as: U.K. Patent No.861,138; U.S. Pat. Nos. 3,632,345, 3,928,041, 3,958,993 and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Pat. Nos. 1,939,231; 2,181,944; 2,333,106; and 4,126,461; German OLS No.2,644,194 and German OLS No.2,650,764. Typically, such couplers are resorcinols or m-aminophenols that form black or neutral products on reaction with oxidized color developing agent.

It may be useful to use a combination of couplers any of 25 which may contain known ballasts or coupling-off groups such as those described in U.S. Pat. Nos. 4,301,235; 4,853, 319 and 4,351,897. The coupler may contain solubilizing groups such as described in U.S. Pat. No. 4,482,629.

Typically, couplers are incorporated in a silver halide 30 emulsion layer in a mole ratio to silver of 0.1 to 1.0 and generally 0.1 to 0.5. Usually the couplers are dispersed in a high-boiling organic solvent in a weight ratio of solvent to coupler of 0.1 to 10.0, typically 0.1 to 2.0 and usually 0.1 to 0.6, although direct dispersions are sometimes employed.

The invention materials may also be used in association 35 with materials that accelerate or otherwise modify the processing steps e.g. of bleaching or fixing to improve the quality of the image. Bleach accelerator releasing couplers such as those described in EP 193,389; EP 301,477; U.S. Pat. Nos. 4,163,669; 4,865,956; and 4,923,784, may be useful.

Also contemplated is use of the compositions in association 40 with nucleating agents, development accelerators or their precursors (UK Patent 2,097,140; U.K. Patent 2,131,188); electron transfer agents (U.S. Pat. Nos. 4,859,578; 4,912, 025); antifogging and anti color-mixing agents such as 45 derivatives of hydroquinones, aminophenols, amines, gallic acid; catechol; ascorbic acid; hydrazides; sulfonamidophenols; and non color-forming couplers.

It is contemplated that the concepts of the present invention may be employed to obtain reflection color prints as 50 described in *Research Disclosure*, November 1979, Item 18716, available from Kenneth Mason Publications, Ltd, Dudley Annex, 12a North Street, Emsworth, Hampshire P0101 7DQ, England, incorporated herein by reference. Materials of the invention may be coated on pH adjusted support as described in U.S. Pat. No. 4,917,994; on a support with reduced oxygen permeability (EP 553,339); with epoxy solvents (EP 164,961); with nickel complex stabilizers (U.S. Pat. Nos. 4,346,165; 4,540,653 and 4,906,559 for example); with ballasted chelating agents such as those in U.S. Pat. No. 4,994,359 to reduce sensitivity to polyvalent cations such as 55 calcium; and with stain reducing compounds such as described in U.S. Pat. No. 5,068,171. Other compounds useful in combination with the invention are disclosed in Japanese Published Applications described in Derwent Abstracts having accession numbers as follows: 90-072,629, 90-072,630; 90-072,631; 90-072,632; 90-072,633; 90-072, 634; 90-077,822; 90-078,229; 90-078,230; 90-079,336; 90-079,337; 90-079,338; 90-079,690; 90-079,691; 90-080,

60 65 70 75 80 85 90 95 100

487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

Conventional radiation-sensitive silver halide emulsions can be employed in the practice of this invention. Such emulsions are illustrated by *Research Disclosure*, Item 38755, September 1996, I. Emulsion grains and their preparation.

Especially useful in this invention are tabular grain silver halide emulsions. Tabular grains are those having two parallel major crystal faces and having an aspect ratio of at least 2. The term "aspect ratio" is the ratio of the equivalent circular diameter (ECD) of a grain major face divided by its thickness (t). Tabular grain emulsions are those in which the tabular grains account for at least 50 percent (preferably at least 70 percent and optimally at least 90 percent) of the total grain projected area. Preferred tabular grain emulsions are those in which the average thickness of the tabular grains is less than 0.3 micrometer (preferably thin—that is, less than 0.2 micrometer and most preferably ultrathin—that is, less than 0.07 micrometer). The major faces of the tabular grains can lie in either {111} or {100} crystal planes. The mean ECD of tabular grain emulsions rarely exceeds 10 micrometers and more typically is less than 5 micrometers.

In their most widely used form tabular grain emulsions are high bromide {111} tabular grain emulsions. Such emulsions are illustrated by Kofron et al U.S. Pat. No. 4,439,520, Wilgus et al U.S. Pat. No. 4,434,226, Solberg et al U.S. Pat. No. 4,433,048, Maskasky U.S. Pat. Nos. 4,435,501, 4,463,087 and 4,173,320, Daubendiek et al U.S. Pat. Nos. 4,414,310 and 4,914,014, Sowinski et al U.S. Pat. No. 4,656,122, Piggie et al U.S. Pat. Nos. 5,061,616 and 5,061,609, Tsaur et al U.S. Pat. Nos. 5,147,771, '772, '773, 5,171,659 and 5,252,453, Black et al U.S. Pat. Nos. 5,219,720 and 5,334,495, Delton U.S. Pat. Nos. 5,310,644, 5,372,927 and 5,460,934, Wen U.S. Pat. No. 5,470,698, Fenton et al U.S. Pat. No. 5,476,760, Eshelman et al U.S. Pat. Nos. 5,612,175 and 5,614,359, and Irving et al U.S. Pat. No. 5,667,954.

Ultrathin high bromide {111} tabular grain emulsions are illustrated by Daubendiek et al U.S. Pat. Nos. 4,672,027, 4,693,964, 5,494,789, 5,503,971 and 5,576,168, Antoniades et al U.S. Pat. No. 5,250,403, Olm et al U.S. Pat. No. 5,503,970, Deaton et al U.S. Pat. No. 5,582,965, and Maskasky U.S. Pat. No. 5,667,955.

High bromide {100} tabular grain emulsions are illustrated by Mignot U.S. Pat. Nos. 4,386,156 and 5,386,156.

High chloride {111} tabular grain emulsions are illustrated by Wey U.S. Pat. No. 4,399,215, Wey et al U.S. Pat. No. 4,414,306, Maskasky U.S. Pat. Nos. 4,400,463, 4,713, 323, 5,061,617, 5,178,997, 5,183,732, 5,185,239, 5,399,478 and 5,411,852, and Maskasky et al U.S. Pat. Nos. 5,176,992 and 5,178,998. Ultrathin high chloride {111} tabular grain emulsions are illustrated by Maskasky U.S. Pat. Nos. 5,271,858 and 5,389,509.

High chloride {100} tabular grain emulsions are illustrated by Maskasky U.S. Pat. Nos. 5,264,337, 5,292,632, 5,275,930 and 5,399,477, House et al U.S. Pat. No. 5,320,938, Brust et al U.S. Pat. No. 5,314,798, Szajewski et al U.S. Pat. No. 5,356,764, Chang et al U.S. Pat. Nos. 5,413,904 and 5,663,041, Oyamada U.S. Pat. No. 5,593,821, Yamashita et al U.S. Pat. Nos. 5,641,620 and 5,652,088, Saitou et al U.S. Pat. Nos. 5,652,089, and Oyamada et al U.S. Pat. No. 5,665,530. Ultrathin high chloride {100} tabular grain emulsions can be prepared by nucleation in the presence of iodide, following the teaching of House et al and Chang et al, cited above.

The emulsions can be surface-sensitive emulsions, i.e., emulsions that form latent images primarily on the surfaces

of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent. Tabular grain emulsions of the latter type are illustrated by Evans et al U.S. Pat. No. 4,504,570.

Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye. If desired "Redox Amplification" as described in *Research Disclosure* XVIII-B(5) may be used.

With negative-working silver halide, the processing step described above provides a negative image. One type of such element, referred to as a color negative film, is designed for image capture. Speed (the sensitivity of the element to low light conditions) is usually critical to obtaining sufficient image in such elements. Such elements are typically silver bromoiodide emulsions and may be processed, for example, in known color negative processes such as the Kodak C-41 process as described in *The British Journal of Photography Annual* of 1988, pages 191-198. If a color negative film element is to be subsequently employed to generate a viewable projection print as for a motion picture, a process such as the Kodak ECN-2 process described in the H-24 Manual available from Eastman Kodak Co. may be employed to provide the color negative image on a transparent support. Color negative development times are typically 3' 15" or less and desirably 90 or even 60 seconds or less.

Another type of color negative element is a color print. Such an element is designed to receive an image optically printed from an image capture color negative element. A color print element may be provided on a reflective support for reflective viewing (e.g. a snap shot) or on a transparent support for projection viewing as in a motion picture. Elements destined for color reflection prints are provided on a reflective support, typically paper, employ silver chloride emulsions, and may be optically printed using the so-called negative-positive process where the element is exposed to light through a color negative film which has been processed as described above. The print may then be processed to form a positive reflection image using, for example, the Kodak RA-4 process as generally described in PCT WO 87/04534 or U.S. Pat. No. 4,975,357. Color projection prints may be processed, for example, in accordance with the Kodak ECP-2 process as described in the H-24 Manual. Similarly, back-lit image transparencies may be prepared for display purposes. Color print development times are typically 90 seconds or less and desirably 45 or even 30 seconds or less.

The above emulsions are typically sold with instructions to process using the appropriate method such as the mentioned color negative (Kodak C-41), color print (Kodak RA-4), or reversal (Kodak E-6) process.

Preferred color developing agents are p-phenylenediamines such as:

4-amino-N,N-diethylaniline hydrochloride,  
4-amino-3-methyl-N,N-diethylaniline hydrochloride,  
4-amino-3-methyl-N-ethyl-N-(2-methanesulfonamidoethyl)aniline sesquisulfate hydrate,  
4-amino-3-methyl-N-ethyl-N-(2-hydroxyethyl)aniline sulfate,

4-amino-3-(2-methanesulfonamido-ethyl)-N,N-diethylaniline hydrochloride and

4-amino-N-ethyl-N-(2-methoxyethyl)-m-toluidine di-p-toluene sulfonic acid.

Development is usually followed by the conventional steps of bleaching, fixing, or bleach-fixing, to remove silver or silver halide, washing, and drying.

The entire contents of the patents and other publications cited in this specification are incorporated herein by reference.

#### PHOTOGRAPHIC EXAMPLES

##### Preparation of Photographic Elements

Dispersions of the couplers were prepared as below. In one vessel, the coupler, coupler solvent, stabilizer(s), and 15 ethyl acetate were combined and warmed to dissolve. To this solution was added gelatin, surfactant, and water. After manual mixing the mixture was passed three times through a Gaulin colloid mill.

The photographic elements were prepared by coating the 20 following layers in the order listed on a resin-coated paper support:

| 1st layer                                                      |                          |
|----------------------------------------------------------------|--------------------------|
| Gelatin                                                        | 3.23 g/m <sup>2</sup>    |
| 2nd layer                                                      |                          |
| Gelatin                                                        | 1.83 g/m <sup>2</sup>    |
| Coupler                                                        | 0.50 mmol/m <sup>2</sup> |
| Dibutylphthalate                                               | 0.54 g/m <sup>2</sup>    |
| Stabilizer ST-1                                                | 0.27 g/m <sup>2</sup>    |
| Stabilizer AST-1                                               | 0.27 g/m <sup>2</sup>    |
| Green sensitized AgCl emulsion                                 | 0.17 g/m <sup>2</sup>    |
| 3rd layer                                                      |                          |
| Gelatin                                                        | 1.34 g/m <sup>2</sup>    |
| 2-(2H-benzotriazol-2-yl)-4,6-bis-(1,1-dimethyl-propyl)phenol   | 0.73 g/m <sup>2</sup>    |
| Tinuvin 326™ (Ciba-Geigy)                                      | 0.13 g/m <sup>2</sup>    |
| Hexanoic acid,2-ethyl-,1,4-cyclohexanediyl bis(methylene)ester | 0.29 g/m <sup>2</sup>    |
| 1,4-Benzenediol,2,5-bis(1,1,3,3-tetramethylbutyl)-             | 0.18 g/m <sup>2</sup>    |
| 4th layer                                                      |                          |
| Gelatin                                                        | 1.40 g/m <sup>2</sup>    |
| Bis(vinylsulfonylmethyl) ether                                 | 0.14 g/m <sup>2</sup>    |

The photographic elements were given stepwise exposures to blue light and processed as follows at 35° C.:

|                      |                      |
|----------------------|----------------------|
| Developer            | 45 seconds           |
| Bleach-Fix           | 45 seconds           |
| Wash (running water) | 1 minute, 30 seconds |

The developer and bleach-fix were of the following compositions:

| Developer                           |           |
|-------------------------------------|-----------|
| Water                               | 700.00 mL |
| Triethanolamine                     | 12.41 g   |
| Blankophor REU™ (Mobay Corp.)       | 2.30 g    |
| Lithium polystyrene sulfonate (30%) | 0.30 g    |
| N,N-Diethylhydroxylamine (85%)      | 5.40 g    |
| Lithium sulfate                     | 2.70 g    |

-continued

|                                                                                                         |           |
|---------------------------------------------------------------------------------------------------------|-----------|
| 4-amino-3-methyl-N-ethyl-N-(2-methanesulfonamidoethyl)aniline sesquisulfate hydrate                     | 5.00 g    |
| 1-Hydroxyethyl-1,1-diphosphonic acid (60%)                                                              | 0.81 g    |
| Potassium carbonate, anhydrous                                                                          | 21.16 g   |
| Potassium chloride                                                                                      | 1.60 g    |
| Potassium bromide                                                                                       | 7.00 mg   |
| Water to make                                                                                           | 1.00 L    |
| pH @ 26.7° C. adjusted to 10.04 +/- 0.05                                                                |           |
| <u>Bleach-Fix</u>                                                                                       |           |
| Water                                                                                                   | 700.00 mL |
| Solution of ammonium thiosulfate (54.4%) + ammonium sulfite(4%)                                         | 127.40 g  |
| Sodium metabisulfite                                                                                    | 10.00 g   |
| Acetic acid (glacial)                                                                                   | 10.20 g   |
| Solution of ammonium ferric ethylenediaminetetraacetate (44%) + ethylenediamine tetraacetic acid (3.5%) | 110.40 g  |
| Water to make                                                                                           | 1.00 L    |
| pH @ 26.7° C. adjusted to 5.50 +/- 0.10                                                                 |           |

#### PHOTOGRAPHIC TESTS

Magenta dyes were formed upon processing. The following photographic characteristics were determined:  $D_{max}$  (the maximum density to green light); Speed (the relative log exposure required to yield a density to green light of 1.0); 30 and Contrast (the ratio (S-T)/0.6, where S is the density at a log exposure 0.3 units greater than the Speed value and T is the density at a log exposure 0.3 units less than the Speed value).

The element of this invention provided comparable and acceptable values for  $D_{max}$ , Contrast, Speed, and other photographic properties when they are coated, exposed in a controlled manner, and processed as above.

The elements were also subjected to accelerated testing under high intensity daylight conditions to determine the portion of the dye that is lost during light exposure. Various inventive and control couplers were substituted for the coupler in layer 2 and each was tested as described above. It was found that the selection of  $R_1$  having more than 10 carbon atoms served to improve the light fastness of areas where magenta dye is formed. Table I contains dye fade data corresponding to the density change observed from processed strips at an initial density of 1.0 when the strips are subjected to a high intensity light fade by exposure to the light of a xenon arc lamp at an intensity of 50,000 lux.

TABLE I

|    |        |         | Dye Fade<br>3 wk<br>from 1.0 |
|----|--------|---------|------------------------------|
|    | Sample | Coupler | Type                         |
| 60 | 1      | M1      | Inv                          |
|    | 2      | C1      | Comp                         |
|    | 3      | M19     | Inv                          |
|    | 4      | C2      | Comp                         |
|    | 5      | M20     | Inv                          |
|    | 6      | C3      | Comp                         |
|    | 7      | M21     | Inv                          |
| 65 | 8      | M11     | Inv                          |

The comparison couplers were as follows:



As can be seen from the data, the presence of more than 10 carbon the R<sub>1</sub> group served to improve the dye light stability of the magenta dye. Using comparison couplers C1, C2, or C3, the dye fade ranged from 17–20% of the original dye density. When the R<sub>1</sub> substituent is selected in accordance with the invention, the loss is reduced to a range of 9 to 13%, an improvement of approximately 50%.

What is claimed is:

1. A photographic element comprising a light sensitive silver halide emulsion layer having in association therewith at least one dye-forming coupler of Formula (1a):



wherein:

R<sub>1</sub> is an alpha-branched alkyl group with greater than 10 carbon atoms;

R<sub>5</sub>, R<sub>6</sub>, R<sub>7</sub>, and R<sub>8</sub> are each independently a hydrogen atom or a substituent;

Z is a hydrogen atom or a group which can be split off by the reaction of the coupler with an oxidized color developing agent.

2. The element of claim 1 wherein each of R<sub>5</sub>, R<sub>6</sub>, R<sub>7</sub>, and R<sub>8</sub> are hydrogen.

3. The element of claim 1 in which Z is a substituted alkylthio group.

4. The element of claim 1 wherein the light sensitive silver halide layer additionally contains a first light stabilizer having Formula (ST-I):

(ST-I)



wherein R<sub>b</sub> is a substituent, n is an integer from 0 to 4, R<sub>d</sub> and R<sub>e</sub> are each independently hydrogen atoms or alkyl groups, provided that any of the groups R<sub>b</sub>, R<sub>d</sub> and R<sub>e</sub> may be joined together to form a ring.

5. The element of claim 1 wherein the light sensitive silver halide layer additionally contains a first light stabilizer having formula (ST-II):

C3

(ST-II)



wherein R<sub>3</sub> represents an aryl group or a heterocyclic group; Z<sub>1</sub> and Z<sub>2</sub> independently represent an alkylene group having 1 to 3 carbon atoms provided that the total number of carbon atoms in the ring is 3 to 6; and q is an integer of 1 or 2.

6. The element of claim 1 wherein the light sensitive silver halide layer additionally contains a first light stabilizer having Formula (ST-IV):



wherein R<sub>a</sub> is an alpha-branched alkyl group, R<sub>b</sub> is a substituent and n is an integer from 0 to 4.

7. The element of claim 4 wherein the light sensitive silver halide emulsion layer additionally contains a light stabilizer having Formula (AST):

AST



wherein

each R<sub>4</sub> group independently represents an alkyl or alkoxy group of 1 to 32 carbon atoms and p is 1 to 4;

Y is —NHSO<sub>2</sub>— or —SO<sub>2</sub>NH—, and

R<sub>5</sub> is an alkyl group of 1 to 16 carbon atoms.

8. The element of claim 7 wherein n is 0.

9. The element of claim 1 wherein the coupler is dispersed in droplets of coupler solvent that additionally contain a stabilizer where the amount of dye-forming coupler of Formula (1a) is 5% to 40% of the total amount of the coupler, stabilizer and coupler solvent.

10. The element of claim 9 wherein the total amount of dye-forming coupler of Formula (1a) is 7% to 15% of the total amount of the coupler, stabilizer and coupler solvent.

11. A multicolor photographic element, comprising: a support bearing at least one blue light-sensitive silver halide

**23**

emulsion layer having associated therewith at least one yellow dye-forming coupler, at least one red light-sensitive silver halide emulsion layer having associated therewith at least one cyan dye-forming coupler, and at least one green light-sensitive silver halide emulsion layer having associated therewith at least one magenta dye-forming coupler of Formula (1a):

**24**

R<sub>1</sub> is an alpha-branched alkyl group with greater than 10 carbon atoms;

R<sub>5</sub>, R<sub>6</sub>, R<sub>7</sub>, and R<sub>8</sub> are each independently a hydrogen atom or a substituent;

<sup>5</sup> Z is a hydrogen atom or a group which can be split off by the reaction of the coupler with an oxidized color developing agent.

<sup>10</sup> 12. The element of claim 11 wherein the halide content of the emulsion is at least 90 mole % chloride.

13. The element of claim 11 wherein the support is a reflective support.

<sup>15</sup> 14. A process for forming an image in the element of claim 1 after the element has been imagewise exposed to light, comprising contacting the exposed element with a color developing compound.

15. The element of claim 14 wherein the color developing compound is a p-phenylenediamine compound.

\* \* \* \* \*

wherein: